

May 10, 1932.

G. C. CARSON

1,857,494

METHOD AND MEANS FOR TREATING SULPHIDE ORES AND  
THE PRODUCTION OF SULPHURIC ACID THEREBY

Filed Oct. 6, 1925

2 Sheets-Sheet 1



Invention

GEORGE CAMPBELL CARSON

by Miller & Boyken

Attorneys

May 10, 1932.

G. C. CARSON

1,857,494

METHOD AND MEANS FOR TREATING SULPHIDE ORES AND  
THE PRODUCTION OF SULPHURIC ACID THEREBY

Filed Oct. 6, 1925

2 Sheets-Sheet 2



Inventor:  
GEORGE CAMPBELL CARSON  
by Miller & Boyken  
Attorneys.

## UNITED STATES PATENT OFFICE

GEORGE CAMPBELL CARSON, OF LOS ANGELES, CALIFORNIA

## METHOD AND MEANS FOR TREATING SULPHIDE ORES AND THE PRODUCTION OF SULPHURIC ACID THEREBY

Application filed October 6, 1925. Serial No. 60,840.

Generally stated, my invention relates to a method of and apparatus for treating mixed sulphide ores for the ultimate recovery of the metal values therein and the production of sulphuric acid, the ores, in finely pulverized condition, being caused to pass in one direction in a stream of acid solvent which is flowing in the opposite direction whereby sulphides of the metals are converted into the corresponding sulphates which become dissolved in the stream and pass with it in one direction while the unconverted sulphides and the insolubles pass in the up-stream direction, finally leaving the stream at or near its source. Since metal sulphides vary in respect of the ease with which they yield to the acid attack, some are sulphated, and the sulphates dissolved, almost as soon as they contact with the acid solvent, while others are highly resistant and are, consequently, carried far up-stream before they yield to the acid attack if they yield at all. The sulphates in the stream thus tend to separate from one another; and their substantially complete separation is made possible in practice by reason of the fact that a sulphate in solution is reduced to its sulphide form by coming into contact with a sulphide which is more easily sulphated, being thus precipitated as a solid which is again advanced up the stream into the region where it was first sulphated, and where it is again sulphated and the sulphate dissolved. By these alternating reactions and precipitations, which may take place again and again, the sulphates in the stream become so effectually separated that they may be individually treated, either while in the stream or after withdrawal therefrom, for recovery of their metal values. One feature of the invention, therefore, consists in the chemical treatment of the metal sulphides in such a manner as to effect the separation of their dissolved sulphates.

More specifically, the method consists in the passage of the pulverized mixed sulphides up a stream of acid (principally  $H_2SO_4$ ) solvent and through a train of reaction vessels through which the solvent is flowing, preferably by gravity. The sulphides enter the stream at or near one end of the train while the acid enters, or is formed, at or near the opposite end thereof and flows through the train and out at or near the point where the sulphides enter. As will be seen, the products of the method give to the stream its solvent power, the principal one of which is the anhydride  $SO_3$  which, when introduced into the stream at any desired point, replenish or maintain the strength of the acid. Near the source of the stream the acid is maintained relatively strong in order effectually to attack sulphides which have resisted the attack of the weaker acid farther down stream. The acid grows weaker as it expends itself in its attacks, except as it is replenished as above stated, until it is substantially exhausted at or near the exit of the solvent stream. As it passes along through the train of vessels, it meets successively sulphides in the reverse order of their susceptibility to attack, those more susceptible having already been oxidized and their sulphates entered into the solution. While, therefore, the solvent gradually weakens in its acid content as it passes down the stream, the dissolved sulphates therein gradually increase in quantity until, at or near the end of the train, the liquid is saturated therewith. In fact, since the reactions are generally exothermic, the temperature at that point is such that the solution may be said to be supersaturated; for if it were cooled, some of the sulphates would be precipitated as crystals, the liquid being unable to carry them in solution at the reduced temperature. These sulphates are treated for the recovery of their metal values or are reduced to sulphides and discharged as such as products, while the insolubles, such as  $PbSO_4$ ,  $Ag_2SO_4$ ,  $M$  and  $SiO_2$ , are discharged at the other end of the train for separation in a known manner. ( $M$  being symbolic of an insoluble metal.)

In carrying out the process, various steps may be resorted to at different stages, dependent upon the local ore content or the predominance of a specific metal or metal compound, so as to adapt the process to the treatment of complex sulphide ores of all kinds; and various treatments are given some of the

finally separated metallic salts either for returning part of their constituents to the train to carry on the process or as a further product of the process.

5 My process may be carried out through a batch system of treatment wherein the progressive reactions take place in separate tanks to which the reaction solutions and precipitates are progressively transferred in the required directions or, better, in a system which is continuous in so far as the general treatment is concerned, being contributed to, when expedient, by individual treatment of some of the derivatives.

10

15 In carrying out my method along the lines last suggested, I prefer to arrange the various reaction vessels to provide a flow, as revealed in the flow sheet shown in Fig. 1 of the drawings hereto, and in which the reaction vessels in the main train take the preferred form which is shown in vertical section in Fig. 2 of the drawings, and of which latter figure, Figs. 3 and 4 are details.

20

In the flow sheet, the general travel of the liquid or solvent is in the direction of the arrow A. Starting from vessel 98, it passes through the successively lower-numbered vessels of the main train to the one marked 50, and thence through the special-treatment vessels 39 to 46. The flow of the ore material under treatment is in the opposite direction, as indicated by the arrow B, beginning with a charge of material to vessel 50. A large part of this material is oxidized and dissolved while passing through the train of reaction vessels and so never reaches the vessel 98.

The vessels 50 to 98 inclusive are designed to effect this counter current flow of material and solvent. The auxiliary row of vessels 29 to 35 are successive agitators, while the other vessels shown are precipitation tanks, filters, etc., as will appear in the description of the reactions to follow.

45 In Fig. 2, which illustrates the preferred form of construction of vessels 50 to 98, two adjacent vessels are shown. These vessels, which are properly supported on a foundation 1, comprise a vitreous or acid-proof inner shell 2, made in sections, as indicated, cemented together with an acid-proof cement and covered by suitable lids 3. Each vessel is provided with an overflow discharging to the lower part of the next vessel 50 through a suitable tile 4, the upper part of the overflow widening and terminating in a weir 5 which preferably extends across the vessel. The successive weirs are gradually lower and lower as the train of vessels proceeds in the direction of arrow A. A liquid 6 introduced into one vessel will, therefore, flow successively through all of the vessels having lower numbers from the top of one to the bottom of the next. The lower portion 60 65 2' is made conical, as shown, so as to concen-

trate toward the center any pulverulent material introduced into the vessel for reaction with the liquid.

The conical lower portion 2' is preferably formed of two sections, each of a single vitreous member and with the upper one, as shown in plan in Fig. 3 and in vertical section in Fig. 4, comprising an outer ring with ribs supporting a central sleeve 7 which, when assembled in the vessel, in turn supports vertical sleeve sections 8 and 9, the latter being open at the upper end and having, in addition, lateral passages 10. 70 75

Below the lower end of the conical section 2' is a removable bottom section 11, which is seated against a gasket 12 and is held in place by jack screws 13. This removable bottom, which provides for cleaning and repairing, houses a duct 14, through which the solids from one vessel are led for upward discharge to the next adjacent vessel through a pipe 15, the material being forced upward by a pressure jet arranged under the pipe. 80 85

The upper end of the pipe 15 passes through the wall of the next vessel and terminates in a bell or hood 25, which is inverted over the open end of sleeve 9 so as to discharge solid material from the pipe into the sleeve, while, positioned under the lower sleeve section, is a pressure elevating jet 26 which agitates and forces the solid matter 114 and liquid 6 upwardly to meet the downcoming stream of material from the hood 25. This results in a lateral ejection of the thoroughly mixed material and liquid through the sleeve passages 10, the circulation being as indicated by the arrows in Fig. 2. 100

In carrying out my process, the jets 16 and 26 are operated by sulphuric anhydride, air or a combination of both the anhydride and air, sulphuric acid, solution ferricsulphate, or any other suitable agency, and the ensuing reaction usually maintains the temperature of the vessel's contents at or near the boiling point. Where, however, due to the nature of the material under treatment or to weakness of the acid, the temperature of the contents falls too low, steam is also introduced through the jets; and, in some of the vessels, additional steam coils may be used, as shown at 27 in Fig. 2. These coils may open at the lower end to the vessel, as indicated at 27', or they may be closed at that end, all depending on whether the addition of more water to the contents is desirable.

The air which may be driven up through the jets 16 and 26 is not merely an agitating and propelling medium, since it aids in the oxidation and sulphatization of the sulphides. It readily attacks the sulphides pyrrhotite and marcasite and converts the ferrous sulphate produced therefrom into ferric sulphate. This ferric sulphate is one of the most powerful chemical agents known; and when formed as just stated, or when it is

formed and introduced into the stream, as hereinafter described, it oxidizes any hydrogen sulphide present and with which it contacts into sulphuric acid, being changed thereby back to ferrous sulphate. Since the 5 hydrogen sulphide interferes with the reactions by precipitating sulphides from sulphates already formed and, being noxious, its escape into the air is objectionable, it will be 10 seen that the air injected through the jets 15 performs an important function.

Having thus given a general description of the main apparatus units, my process in the treatment of complex sulphide ores will now 15 be set forth.

The mixed or complex sulphide ores, unroasted and otherwise untreated except by crushing until they are in a fine state of division, preferably such as flotation concentrates, are supplied from a source 28, first, in 20 moderate quantity, to the vessel 50 at the lower end of the train. In some circumstances it may be desirable to introduce the ores at other points as well, and Fig. 1 indicates that 25 they may be introduced at vessels 52, 58, 61, 63 and 72. Of course, these particular vessels are designated for illustration only, as the ores may enter the train at any point where their presence is required or may be 30 advantageous, as will be more particularly explained hereinafter. The reaction liquid is introduced at or near the upper end of the train, from which it flows through the vessels of lower numbers in series toward the 35 vessel 50. The liquid is caused to fill the vessels and overflow the weirs 5, while the ores are introduced at the tops of the vessels, as by dropping them through gate-controlled chutes, all as indicated in Fig. 2. The ores 40 fall upon the surface of the liquid and settle downwardly, being violently agitated in the vessels by the jets 26 and transferred in an up-stream direction by the jets 16. The finer particles of some of the sulphides yield 45 almost immediately to the acid attack, and the resulting effervescence assists in agitating the contents of the vessels.

But before a proper appreciation of the reactions can be obtained, it is necessary to consider all of the vessels in the train proper, as 50 well as the auxiliary apparatus, as working to their maximum chemical efficiency, since the relative changes in the traveling solids and the oppositely traveling liquids depend 55 thereon. Therefore, the various reaction vessels 50 to 94 must be considered as containing, in their ascending numerical order, sulphide ores of increasing resistance to the acid attack, while the vessels 95 to 98 contain 60 insoluble matter only. The chemical solvent, the principal reaction agent of which is sulphuric acid, must be considered as being weakest in dissolved minerals (in the form 65 of sulphates) at the vessel 94, as flowing in 70 the direction of the arrow A, and as progres-

sively increasing in its sulphate content to the point of saturation of supersaturation at the vessel 50, the sulphides being passed in the direction of the arrow B counter to the flow 70 of the liquid, as has been stated.

For initially starting the operation, batches of ore and liquid in the proper relative amounts and consistencies may be introduced into the various vessels; or a quantity of the sulphide ore material may be delivered to each 75 vessel through its feed chute, or otherwise, and, without operating the jets 16, the solvent run slowly through the successive vessels, with agitation by the jets 26, until the proper conditions are obtained. 80

Assuming that the liquid is in the condition of increasing solutes toward the vessel 50; that the sulphide in the train are of progressively increasing resistance to oxidation from the vessels 50 to 94; that the liquid is maintained at substantially the boiling temperature, and that the materials charged into the vessels consist principally of a mixture of the sulphides of lead, copper, iron and zinc, together with their usually associated sulphides, such as minor quantities of the sulphides of cadmium, arsenic, antimony, bismuth, etc., as well as a certain amount of the precious metals, silica and other insoluble material, the operation and some of the principal 90 reactions will now be set forth. 95

The material is charged into the train at vessel 50 and, if desired, at other points as well, while the stream of liquid is started by the introduction of wash water into the vessels 98 to 95 and of acid or acid-forming compounds into the vessel 94. Water may be added at other points where required or advantageous, and the same is true of the acid or acid-forming compounds. The jets 16 are operated to carry the material from vessel to vessel while agitation is effected by the jets 26 and by effervescence due to the reactions, as stated. The insoluble compounds pass successively through the vessels 95 to 98 where they are washed, the wash water, and any acid that it has removed from the insolubles, passing to vessel 94 and on through the train. After being thus washed, the insolubles are 100 filtered at 36 and deposited at 37 as a product, consisting usually of a mixture of insoluble sulphates, etc., as designated on the flow sheet. 105

The reacting agent introduced at 94 and elsewhere, as through the jets 16 and 26, may be simply the sulphuric anhydride ( $\text{SO}_3$ ), obtained as hereinafter described, or ferric sulphate and air may also be used. On meeting the wash water from the vessels 98 to 95, the  $\text{SO}_3$  is converted into  $\text{H}_2\text{SO}_4$ . Or the reacting agent may be both  $\text{SO}_3$  and  $\text{H}_2\text{SO}_4\text{H}_2\text{O}$ , the  $\text{H}_2\text{SO}_4\text{H}_2\text{O}$  being also a product of the method, as is also to be described. 115 120 125

Wherever acid is introduced and reaction takes place, heat is evolved; and, if it were 130

all introduced at one point the temperature there would rise excessively. Therefore, the acid is added at such points and in such amounts as will maintain the requisite strength and temperature of the solvent. Preferably, the strength of the acid is gradually increased in the vessels 93, 92, etc., thus bringing the solution to the required strength without unduly raising the temperature at any point. The solution should have a temperature approximating the boiling point and a strength sufficient for attacking the most resistant sulphides which it is intended shall yield to it.

15 As the acid solution flows from vessel to vessel in the direction of the vessel 50, it meets a stream of sulphide material traveling through it in the opposite direction, the material in the vessels of lower numbers containing the sulphides most susceptible to acid attack. While the sulphides in the higher numbered vessels are much more resistant to such attack, the acid therein is stronger and some of the sulphides are sulphated and the sulphates are dissolved. These sulphates flow down the stream and presently meet some sulphide coming in the opposite direction which is more easily sulphated than was the sulphide from which the dissolved sulphate was formed. For example, copper sulphate formed and dissolved in a vessel having a higher number travels with and as part of the stream until it meets zinc sulphide. At once, the copper sulphate is converted to the sulphide and is precipitated. These desulphating and precipitating reactions may be represented by the following typical equations:

40 (1)  $\text{CuSO}_4 + \text{ZnS} = \text{CuS} + \text{ZnSO}_4$   
 (2)  $\text{Fe}_2(\text{SO}_4)_3 + \text{H}_2\text{S} = 2\text{FeSO}_4 + \text{H}_2\text{SO}_4 + \text{S}$

When, as in Equation (1), the CuS is formed and is precipitated, it joins the other undissolved materials and is moved back upstream into the same vessel, or into one adjacent thereto, where the  $\text{CuSO}_4$  was first formed. There the CuS is again attacked and sulphated and the sulphate is dissolved. Again this sulphate flows down-stream until some other sulphide is met which changes it back to CuS. This CuS is sent back upstream, as before. Thus, the copper sulphide in the ore charged into the vessel 50, or elsewhere, is moved up-stream by reason of the jets 16, until it reaches the vessel or vessels in which conditions are favorable for sulphating it. Say, for purposes of explanation, these conditions are found in a group of vessels bearing the numbers 80 to 86 inclusive. Through-out their travel from vessel 50 to this group, the CuS in the ore has been agitated with the acid solvent but has remained a sulphide, because the acid has had other more susceptible sulphides to attack or because the acid has been too weak to attack it. By the time it has

reached the said group of vessels, which may be termed the copper sulphate group, almost all the more susceptible sulphides have been sulphated and their dissolved sulphates have passed downstream. Further, as will be noted from Fig. 1, the acid in this group is strengthened, if need be, by the introduction of  $\text{H}_2\text{SO}_4$ , as at vessel 82, or of  $\text{SO}_3$ , as at vessel 83. These particular vessels are designated for illustration only, as the acid may be replenished at any point, as by introducing the strengthening agent or agents through the jets 16 or 26, as hereinbefore stated. Irrespective of the precipitations of the sulphides, as referred to above, and due to their differences in susceptibility to attack, the various sulphides in the stream tend to separate from one another, as is obvious. But the said precipitations and reprecipitations greatly assist in this separation, since they take place in the vessels which are farther down-stream than the groups in which the respective sulphates were formed and in which it is desired they be retained, and the precipitated sulphides are automatically returned to their respective groups where they are again sulphated and dissolved. Thus the various sulphates are accumulated in their respective groups so that they may be individually treated. In the flow sheet it is assumed that the  $\text{CuSO}_4$  is in its most concentrated form in the vessel 83 where it may be electrolyzed out in the vessels themselves or may be passed direct to electrolytic cells, as at 99, for the production of electrolytic copper, the spent electrolyte being returned to the train, as at vessel 73. This direct method of recovery of the metal values is preferably used where the copper content in the ore is relatively small. If the copper content is large, I prefer to by-pass a portion of the solvent sufficient to care for the accumulating copper sulphate, through a train of agitators where it is treated with FeS to precipitate the copper in sulphide form and to produce ferrous sulphate as a preliminary step in the production of ferric sulphate for use in the main reaction train. This latter feature will be described more particularly hereinafter.

Those dissolved sulphates which have not been previously removed from the train pass down the stream, the solution, as it passes along, growing richer and richer in sulphates and weaker and weaker in its power of attack. At the vessel 50 it receives a quantity of fresh sulphide material, and any power which it may have retained is expended thereon, so that the solvent is substantially neutral when it finally leaves the train at said vessel. Owing to the weakness of the acid at and near the lower end of the stream, such reactions as take place generate but a relatively small amount of heat. Consequently, it is desirable to supply such heat as may be necessary to further the reactions and to pre-

vent precipitation of the sulphates through crystallization. This is accomplished by the use of the steam coils 27, or by the injection of steam from the coils at 27 or through the jets 16 or 26.

While the solvent has been growing richer and richer in dissolved sulphates, many of the sulphides have disappeared as such and the remaining solid materials in the train are, in 10 the up-stream direction, progressively more and more resistant to the acid attack, those passing beyond vessel 94 being insoluble.

In Fig. 1 the train of reaction vessels is shown as extending from 50 to 94, which is 15 sufficiently long for purposes of illustration and for many practical operations. The length of the train used would depend upon the materials employed and upon the desired completeness of separation of the sulphates 20 in the stream. Obviously, the longer the train the more completely will this separation be effected.

The attack of the acid on most of the metallic sulphides present in the ore results in 25 the formation of  $H_2S$ . Thus,



Although it is a gas, the  $H_2S$  is absorbed 30 by the solution; and, if it were not removed or converted into other compounds, it would interfere with the sulphating process. In fact, the solution would become so far saturated with it that the metal sulphates would 35 be desulphated substantially as fast as they could be formed. This is shown by Equation (2) or by the following:



It is, therefore, important that the  $H_2S$  be 40 converted into something which will not reduce the sulphates in the solution. Better still if it can be converted into  $H_2SO_4$  and made to strengthen the solvent. Further, there are some conditions in which  $H_2S$  is 45 formed and in which it so disposes itself as greatly to retard the sulphating process. For example, certain sulphides of copper contain arsenic or antimony, and it is difficult to convert them into sulphate form for the reason that the  $H_2S$  evolved adheres to the particles and surrounds them as an envelope or film and thus insulates them from the acid. Any agent introduced into the solution which 50 will attack and remove this envelope will greatly facilitate the attack on these sulphides and prevent them from passing out with the insolubles beyond the vessel 94. The removal of the  $H_2S$ , as such, and its conversion into 55 a beneficial reagent is, therefore, an important feature of my invention which will now be explained.

The sulphides of iron in the train are readily attacked by the acid, the reaction being of 60 the nature shown in Equation (3). But iron

disulphide,  $FeS_2$ , known as primary pyrite, yields very slowly to the  $H_2SO_4$ ; and I have discovered that this pyrite floats as a scum on the surface of the liquid and gives off the noxious  $SO_2$ . This objectionable pyrite may 70 be removed by skimming wherever it may be noted. However, it will not appear in any considerable quantities until the pyrite reaches the relatively strong acid, say at vessels 87 and 88. At that point, as shown in 75 Fig. 1, I arrange a skimmer to remove this scum and pass it into a heater, indicated, where the feeble atoms of S is driven off to a sulphur condenser, also indicated, from which it may be taken as a product of the process. 80 It is the  $FeS$ , left after dissociation in the heater and collected at 38, which becomes of importance in the general process.

This  $FeS$  could, of course, be returned directly to the main train to be sulphated with 85 the other sulphides, but I prefer to use it both in the treatment of certain of the sulphates which have passed beyond the main train at the vessel 50 and also in the preparation of ferric sulphate for use in the train to attack 90 the objectionable  $H_2S$  therein.

As stated, if the copper in the ore is plentiful, I prefer to shunt out a portion of the solvent, the amount so shunted being substantially equal to the copper sulphate which 95 is dissolved in the stream. The object of this shunt of copper-sulphate bearing solution is to separate the copper from the other sulphates and to produce a supply of ferric sulphate from the  $FeS$  produced as above described. Such a shunt is shown connecting the vessels 75 and 76. These vessels differ from those of the main train, since they are adapted merely for agitating the materials and for sending both the liquid and the solids 100 in the same direction through the vessels 29 to 35, as indicated by the arrow in Fig. 1. That is to say, the  $FeS$  and the  $CuSO_4$  enter the vessel 29 and are agitated together with air as they, and the  $CuS$  precipitated thereby, proceed from vessel to vessel. By the time they reach the vessel 35, all the  $FeS$  has been converted to ferrous sulphate and the latter is dissolved while most of the copper sulphate 110 has been changed to  $CuS$  and has been precipitated. Since there may be small amounts of other sulphates present in the solution, such as the sulphates of cadmium, arsenic, antimony and bismuth, all of which are more 115 resistant to the attack of the  $FeS$  than is the copper sulphate, the supply of  $FeS$  to the shunt train of agitators is preferably limited in quantity so as to assure that it will act on the  $CuSO_4$  only. For example; if the 120 quantity of  $CuSO_4$  entering the shunt circuit is theoretically capable of conversion into 2100 pounds of  $CuS$  per minute, the  $FeS$  supplied would be such as to cause but one ton of  $CuS$  to form. In this way, sufficient 125

130

CuSO<sub>4</sub> would always be present in the shunt circuit to prevent the formation of other sulphides therein, and the sulphates of cadmium etc. will pass from the agitators back to the main train at the vessel 75. Furthermore, the use of this limited amount of FeS assures that it will all be used for its intended purpose and that none will remain to pass on with and contaminate the CuS, which it is desired shall be pure. The CuSO<sub>4</sub> which is not thus acted upon by the FeS passes back into the main train at 75 and on down the stream until it meets some sulphide which desulphates it. The CuS thus formed is carried back up-stream to the copper sulphate group of vessels where it is again sulphated. The supernatant liquid containing the FeSO<sub>4</sub> in solution passes from the vessel 35, in part back to the main train at 75 and in part to a storage vessel at 47, while the underflow containing the precipitated CuS passes into a thickener 17 and thence to a filter 18, from which the filter cake is passed to vessels 20 and 21 for treatment with H<sub>2</sub>SO<sub>4</sub> or SO<sub>3</sub>, or a combination of both, to form substantially pure copper sulphate in solution.

This is then passed, through a settler or thickener 22, into electrolytic cells 23 to produce pure electrolytic copper, as indicated at 24, while the spent electrolyte is returned to the main train of vessels wherever required, or is used to sulphate the CuS in the vessels 20 and 21, all as indicated. The filtrate from 18 is passed to the storage vessel 47 along with the solution from vessel 35.

While the treatment of the CuS from the time it leaves the agitator 35 is important from an economic viewpoint, the formation of the FeSO<sub>4</sub> in the shunt circuit is more directly concerned in the method, since it is one of the intermediate compounds obtained in changing the ferrous sulphide, FeS, to ferric sulphate, Fe<sub>2</sub>(SO<sub>4</sub>)<sub>3</sub>. The FeSO<sub>4</sub> is transferred to the vessel 47 along with some H<sub>2</sub>SO<sub>4</sub>, and air is introduced into said vessel, as indicated. If sufficient H<sub>2</sub>SO<sub>4</sub> and O are present, the FeSO<sub>4</sub> is completely converted into ferric sulphate. Thus,



Since, however, the acid accompanying the FeSO<sub>4</sub> has come from the main train at 76 and is largely spent, it is not sufficient for the complete conversion of Equation (5), and only a part of the FeSO<sub>4</sub> is thus converted. The remaining part is both oxidized and hydrolyzed into a basic sulphate of iron as follows:



which breaks up into ferric sulphate and

ferric hydroxide, as appears from the following:



There is thus obtained from reactions (5) and (7) the ferric sulphate required for oxidizing the H<sub>2</sub>S; and this sulphate, after filtration at 48, is led back into the main train at various points, as indicated, where it reacts 75 with the H<sub>2</sub>S in accordance with Equation (2), which is here repeated:



From the above it will be noted that, in carrying out my method in the reaction vessels, two deleterious substances manifest themselves. One is the H<sub>2</sub>S and the other is the scum of the primary pyrite, FeS<sub>2</sub>. By skimming off the latter and dissociating it, I 85 procure FeS, from which there is produced ferric sulphate. By returning the iron content of the pyrite to the train in the form of ferric sulphate, I am enabled to eliminate the H<sub>2</sub>S from the solvent and to build up the 90 acid therein. Thus is one deleterious substance utilized in the removal of the other and in building up the acid.

As has been suggested, a sulphide in the train will not be sulphated if another sulphide which is more susceptible to the acid attack be present with it, as the acid will first attack the latter sulphide. This being true, a sulphide which would otherwise be sulphated in a certain vessel of the train can be caused to remain in the sulphide form and to be carried along to another part of the train by simply introducing some fresh ore with it.

Referring to the flow sheet, the solution, 105 heavily impregnated with sulphates of various kinds, passes from the vessel 50 into a thickener 39 for removal of suspended and settled inert matter. The clear overflow from 39 passes to reaction vessels and 110 thickeners 40 to 42 in which the solution is agitated with another part of the FeS from 38 and sufficient H<sub>2</sub>SO<sub>4</sub> to liberate H<sub>2</sub>S. This H<sub>2</sub>S reacts with the sulphates of Cd, 115 As, Sb, and Bi and precipitates them as sulphides. These reactions are as follows:



These precipitated sulphides, after filtration 120 at 100, are discharged as a mixed product at 101, as indicated.

During the sulphatation of the sulphides in the train, many reactions occur which liberate elemental S, as in Equation (2). This sulphur is carried in suspension in the solution to be removed by the filter 100 and to appear with the mixed products at 101.

The decanted and clear solution from vessels 40 to 42 and filter 100, containing sul-

phates of iron and zinc, passes into vessels 43 to 45, where it is treated with zinc oxide to change the iron sulphates into hydroxides, with the formation of zinc sulphate. Thus,



10 The iron hydroxide, after filtration at 102, is passed as a product to 49, and the filtrate is passed to 45 for final precipitation of its iron content.

15 The ZnO is introduced into the vessel 43 in a limited amount for the reason that, if sufficient were used to precipitate all of the iron there, some of the ZnO would become entangled in the flocculent hydroxide of iron, would remain with it in filtration and would 20 contaminate the precipitate with zinc. To prevent this result, I thicken the first precipitate in vessel 43 and pass the clear solution to 44, and similarly to 45 for further precipitations by fresh charges of ZnO. In the last 25 mentioned vessel I introduce an excess of the ZnO to remove the last trace of iron from the solution and again thicken and transfer the thickenings, which will contain a large amount of ZnO, back into the thickener 43 30 into which the oxide was first introduced.

The solution, after being purified of its iron precipitate by thickening and by the filter at 102, is run into a final thickener 46 and then into crystallizing tanks 103 for cooling. In cooling,  $\text{ZnSO}_4$  crystals are deposited; but the solution with these crystals is withdrawn from the crystallizer before such sulphates as  $\text{MnSO}_4$ , which is more soluble than  $\text{ZnSO}_4$ , begin to deposit. This is further assured by passing the last deposited or the contaminated crystals back to the first stage of the crystallizer for redissolving the more soluble crystals, as  $\text{MnSO}_4$ , thus aiding in forcing out the less soluble  $\text{ZnSO}_4$  crystals. 45 So that substantially pure zinc sulphate crystals are the product of the first stage of the crystallizer. The solution remaining after the  $\text{ZnSO}_4$  crystals have been removed is run into another crystallizer at 104 where it is concentrated to recover the manganese sulphate crystals, which become a product at 50 105.

If the zinc sulphate crystals thus obtained are sufficiently pure, a portion thereof is dissolved and run into electrolytic cells 106 for recovery of metallic zinc at 107, the electrolyte, containing acid, being returned to the main process train as indicated. The remaining and less pure crystals ( $\text{ZnSO}_4 \cdot 7\text{H}_2\text{O}$ ) are passed to a dehydrater 108 where they are heated to drive off the water of crystallization, and the anhydrous zinc sulphate is then passed into a dissociator 109 where it is further heated, in combination with air, to dis-

sociate the sulphuric anhydride,  $\text{SO}_3$ , from the ZnO.

In dissociating the  $\text{ZnSO}_4$  some of its splits up directly into ZnO and  $\text{SO}_3$ , while the rest of it is altered into the basic form  $3\text{ZnO} \cdot 2\text{SO}_3$ , which splits up into 3ZnO,  $2\text{SO}_2$  and O. I thus obtain supplies of  $\text{SO}_3$ ,  $\text{SO}_2$  and O for use in the train of reaction vessels for generating  $\text{H}_2\text{SO}_4$  and supplying the heat of formation. The required amount of the ZnO, 75 which is left after dissociation of the  $\text{ZnSO}_4$ , is used again in the vessels 43 to 45 for precipitating the iron content of the solvent, as has been described. The remaining portion of the ZnO is a by-product of the process.

The mixed gases are freed of dust at 110, given a pressure at 111, and that which is not required in the train process is passed into acid absorbers 112 and manufactured into  $\text{H}_2\text{SO}_4$ , in the known manner, to appear as a 85 product at 113.

The hot water driven off from the  $\text{ZnSO}_4$  is utilized in the manufacture of the  $\text{H}_2\text{SO}_4$  and also as wash water for filtration purposes, as indicated.

95 From the above it will be seen that the invention herein disclosed consists basically in the maintenance of a body or stream of liquid sulphating material, the strength of which increases from one point to another and the transference of the mixed sulphides through said liquid toward the point of its greater strength, whereby the different sulphides are sulphated and dissolved in different parts of the body or stream and from which they may 100 be separately withdrawn for individual treatment. This basic principle is broadly claimed herein. Other claims include this basic principle, but are limited to steps taken in the treatment of certain of the withdrawn 105 sulphates, whereby the basic and acid contents of the sulphates are separated and the latter are fed back into the body or stream or are otherwise used in carrying out the invention. Certain claims which were in the application when filed and which applicant has 110 been required to divide out have now been cancelled without prejudice to applicant's right to reassert them in a divisional application or in divisional applications, to be 115 filed.

I claim:

1. The method of separating the metal values contained in mixed sulphide ores which comprises distributing the sulphides 120 in a flowing stream of sulphating agent in liquid form progressively in the order of their resistance to oxidation by said agent, oxidizing a sulphide of relatively high resistance to form the corresponding sulphate, 125 dissolving said sulphate in said agent, flowing the agent with a portion of the dissolved sulphate therein down stream where there is another sulphide which has less resistance to oxidation to precipitate as sulphide the 130

metal content of the said portion of the dissolved sulphate, moving the precipitated sulphide back into the part of the stream where the sulphate was originally formed, oxidizing the said sulphide and dissolving the sulphate thus formed, whereby the various sulphates are accumulated in different parts of the stream.

2. The method of separating the metal values contained in mixed sulphide ores which comprises maintaining a flowing stream of acidulated sulphating agent in liquid form with the acid strength in the stream increasing in the up-stream direction, introducing the mixed sulphides in comminuted condition into said stream, moving the said sulphides in the said stream in a direction which is counter to the directional flow of the liquid, oxidizing the various sulphides when they reach the respective parts of the stream where the acid strength is sufficient to attack them, thus to convert the sulphides into the corresponding sulphates, dissolving the sulphates in the agent at the parts in the stream where the respective sulphates were thus formed, flowing a portion of a dissolved sulphate down stream away from its point of formation, precipitating as sulphide the metal content of the said portion of the dissolved sulphate, moving the precipitated sulphide back to said point, oxidizing the said precipitated sulphide and dissolving the sulphate thus formed, whereby the sulphate is accumulated in its respective part of the stream.

3. The method of treating mixed and comminuted sulphide ores containing primary pyrite which comprises introducing said ores into a body of sulphating agent in liquid form to convert sulphides therein into the corresponding sulphates with the liberation of hydrogen sulphide in said body, removing the primary pyrite from the body, dissociating said pyrite to form ferrous sulphide, treating said ferrous sulphide to produce ferric sulphate, and introducing the latter to said body to remove the hydrogen sulphide therefrom.

4. The method of treating mixed and comminuted sulphide ores containing primary pyrite which comprises introducing said ores into an elongated body of sulphating agent in liquid form near one end of the body, causing said ores to traverse the said body to convert sulphides therein into the corresponding sulphates with the liberation of hydrogen sulphide in said body, removing from the said body the primary pyrite floating thereon, dissociating said pyrite to form ferrous sulphide, treating said ferrous sulphide to produce ferric sulphate, and introducing the latter to said body to remove the hydrogen sulphide therefrom.

5. The method of treating mixed and comminuted sulphide ores containing primary

pyrite which comprises maintaining a flowing stream of sulphating agent in liquid form, introducing the ores into said stream near the lower end thereof, advancing said ores through the liquid in the up-stream direction, oxidizing certain of the sulphides therein into the corresponding sulphates with the formation of hydrogen sulphide, removing the primary pyrite from the stream, dissociating said pyrite to form ferrous sulphide, treating said ferrous sulphide to produce ferric sulphate, and introducing the latter into said stream to remove the hydrogen sulphide therefrom.

6. The method of treating mixed and comminuted sulphide ores containing primary pyrite which comprises maintaining a flowing stream of sulphating agent in liquid form, introducing the ores into said stream near the lower end thereof, agitating said ores in the liquid and advancing them through the latter in the up-stream direction, oxidizing certain of the sulphides therein into the corresponding sulphates with the formation of hydrogen sulphide, removing from the stream the primary pyrite floating thereon, dissociating said pyrite to form ferrous sulphide, treating said ferrous sulphide to produce ferric sulphate, and introducing the latter into said stream where required to remove the hydrogen sulphide therefrom.

7. The method of separating the metal values contained in mixed sulphide ores which comprises maintaining a flowing stream of acidulated sulphating agent in liquid form with the acid strength in the stream increasing in the up-stream direction, introducing the mixed sulphides in comminuted condition into said stream, discharging into said stream jets of acid-forming agents in such manner as to cause the sulphides in the stream to move in a direction which is counter to the directional flow of the liquid, oxidizing the various sulphides when they reach the respective parts of the stream where the acid strength is sufficient to attack them, thus to convert the sulphides into the corresponding sulphates, and dissolving the sulphates in the stream at the points therein where the respective sulphates were thus formed.

8. The method of separating the metal values contained in mixed sulphide ores which comprises maintaining a flowing stream of acidulated sulphating agent in liquid form with the acid strength in the stream increasing in the up-stream direction, introducing the mixed sulphides in comminuted condition into said stream, discharging into said stream jets of sulphuric anhydride in such manner as to cause the sulphides in the stream to move in a direction which is counter to the directional flow of the liquid, oxidizing the various sulphides when they reach the respective parts of the stream where the acid strength is sufficient

to attack them, thus to convert the sulphides into the corresponding sulphates, dissolving the sulphates in the stream at the points therein where the respective sulphates were thus formed, withdrawing a sulphate from the stream and treating it to obtain sulphuric anhydride for use in the said jets.

9. The method of treating mixed and comminuted sulphide ores containing iron sulphide which comprises maintaining a flowing stream of acidulated sulphating agent in liquid form with the acid strength in the stream increasing in the up-stream direction, introducing the mixed sulphides into said stream, introducing into said stream jets of sulphuric anhydride in such manner as to cause the sulphides to move through the liquid in the up-stream direction, oxidizing the various sulphides when they reach the respective parts of the stream where the acid strength is sufficient to attack them, thus to convert the sulphides into the corresponding sulphates, withdrawing the iron sulphate thus formed from the stream, introducing into the said iron sulphate a metal oxide to convert the iron sulphate into the iron hydroxide with the formation of the sulphate of the said metal, dissociating the latter sulphate with the formation of sulphuric anhydride and using said anhydride in the said jets, as and for the purpose specified.

10. The method of treating mixed and comminuted sulphide ores containing iron sulphide which comprises maintaining a flowing stream of acidulated sulphating agent in liquid form with the acid strength in the stream increasing in the up-stream direction, introducing the mixed sulphides into said stream, introducing into said stream jets of sulphuric anhydride in such manner as to cause the sulphides to move through the liquid in the up-stream direction, oxidizing the various sulphides when they reach the respective parts of the stream where the acid strength is sufficient to attack them, thus to convert the sulphides into the corresponding sulphates, withdrawing the iron sulphate thus formed from the stream, introducing zinc oxide into the said iron sulphate to convert the latter into the iron hydroxide with the formation of zinc sulphate, dissociating the zinc sulphate with the formation of sulphuric anhydride, and using said anhydride in the said jets to move the sulphides up the stream, to maintain the acid strength of the liquid and to furnish the heat necessary to maintain the temperature of the liquid at substantially the boiling point.

11. The method of treating mixed and comminuted sulphide ores containing sulphide of iron and other less easily oxidized sulphides, which comprises maintaining a flowing stream of acidulated sulphating agent in liquid form, introducing the said sulphides into said stream near the lower

end thereof, advancing the sulphides in an up-stream direction whereby they are attacked to form the corresponding sulphates and hydrogen sulphide, dissolving the said sulphates in the liquid stream and flowing them down the stream, treating the mixed sulphates thus produced with ferrous sulphide and sulphuric acid to convert to sulphides all of the sulphates which will react with hydrogen sulphide, removing the precipitated sulphides, treating the resultant liquid containing the iron sulphate with zinc oxide to form zinc sulphate, dissociating the zinc sulphate to produce sulphuric anhydride, and introducing said sulphuric anhydride into the liquid stream to maintain the acid strength therein and to furnish, by the resulting reactions, heat necessary to maintain the liquid at substantially the boiling point.

12. The method of treating mixed and comminuted sulphide ores containing sulphide of iron, which comprises maintaining a flowing stream of acidulated sulphating agent, introducing the said sulphides into said stream near the lower end thereof, advancing the sulphides in an up-stream direction whereby they become oxidized and form the corresponding sulphates, dissolving the said sulphates in the liquid stream and flowing them down the stream, treating the mixed sulphates thus produced to isolate the dissolved iron sulphate, treating the iron sulphate with zinc oxide to form zinc sulphate, dissociating the zinc sulphate to produce sulphuric anhydride, and introducing said sulphuric anhydride into the liquid stream to maintain the acid strength therein.

13. The method of treating mixed and comminuted sulphide ores for the separation of the metal values contained therein which comprises maintaining a body of sulphating agent in liquid form with the acid strength thereof increasing toward one end of the body, introducing the said mixed sulphides into the body where the acid is relatively weak, causing the said sulphides to move through the liquid in the direction of the stronger acid whereby they are attacked by the said agent and the sulphides are converted into the corresponding sulphates at those points where the acid strength is sufficient to attack them, dissolving the sulphates in the liquid and preventing the oxidation of any sulphide at the point where its oxidation would otherwise have occurred by introducing into the liquid at that point another sulphide which is more susceptible to the acid attack, whereby the first mentioned sulphide is caused to be carried farther through the liquid and is more effectually separated from the other sulphides.

14. The method of treating mixed and comminuted sulphide ores for the separation of the metal values contained therein which comprises maintaining a flowing stream of

sulphating agent in liquid form with the acid strength thereof increasing in the up-stream direction, introducing the said mixed sulphides into the stream near the lower end thereof, causing the said sulphides to move up-stream through the liquid whereby they are attacked by the oxidizing agent and the sulphides are converted into the corresponding sulphates at those points in the stream wherein the acid strength is sufficient to attack them, dissolving the sulphates in the stream and preventing the oxidation of any sulphide at the point where its oxidation would otherwise have occurred by introducing into the stream at that point ore containing another sulphide which is more susceptible to the acid attack, whereby the first mentioned sulphide is caused to be carried farther up-stream and is more effectually separated from the other sulphides in the stream.

15. The method of separating the metal values contained in mixed sulphide ores which comprises distributing the sulphides in a flowing stream of sulphating agent in liquid form progressively in the order of their resistance to attack by said agent, oxidizing portions of the various sulphides into the corresponding sulphates, flowing the agent with the dissolved sulphates down the stream from those parts of the latter where the sulphates were formed and into regions where there remains portions of more easily oxidized sulphides, precipitating as sulphides the metal contents of the dissolved sulphates, returning the precipitated sulphides counter current to the flow of the stream until the said sulphides are again oxidized into the respective sulphates, and repeating the cycle of oxidation, dissolution, precipitation and reoxidation until the sulphides are fully oxidized and the dissolved sulphates are separated in the stream.

16. The method of treating mixed sulphide ores in comminuted condition which comprises maintaining an elongated body of oxidizing sulphating liquid the strength of which varies gradually from point to point, introducing said ores into said body where the strength of the liquid is relatively weak, agitating the ores within the liquid and causing them to travel therethrough toward the stronger part of the liquid whereby the sulphides are sulphated and dissolved when they reach those parts of the body where the liquid is strong enough to attack them, withdrawing a dissolved sulphate from that part of the body near which the ores were introduced, treating the said withdrawn sulphate to obtain sulphuric anhydride, and introducing the said anhydride into the said body to maintain the acid strength thereof.

17. The method of separating the metal values contained in mixed sulphide ores which comprises maintaining an elongated body of acidulated sulphating material in

liquid form in which the acid strength varies gradually from one point to another of the body, introducing the mixed sulphides in finely divided condition into said body where the acid strength is relatively weak, discharging into said body jets of acid-forming agents in such manner as to cause the sulphides to move toward the parts of the body where the acid is stronger, sulphating the various sulphides when they reach the respective parts of the body when the acid strength is sufficient to attack them, and dissolving the sulphates in the body at the points therein where the respective sulphates were thus formed.

18. The method of treating mixed and comminuted sulphide ores containing copper sulphide which comprises maintaining a flowing stream of oxidizing sulphating material in liquid form with the acid strength in the stream increasing in the up-stream direction, introducing the mixed sulphides adjacent the lower end of the stream and causing them to move upstream counter to the directional flow of the liquid, sulphating the various sulphides when they reach the respective parts of the stream where the acid is strong enough to attack them with the formation of  $H_2S$ , dissolving the various sulphates at the points in the stream where they were thus formed, withdrawing the sulphate of copper from the stream, introducing  $FeS$  into the copper sulphate to produce  $CuS$  and ferrous sulphate, treating the ferrous sulphate to produce ferric sulphate, and feeding the ferric sulphate into the stream to remove the  $H_2S$  therefrom and to strengthen the acid content of the liquid.

19. The herein described method which comprises maintaining an elongated body of liquid sulphating material the acid strength of which increases gradually in one direction, introducing a mixture containing two sulphides into said material at a point therein where the acid strength is sufficient to attack one but not the other of said sulphides, whereby the said one sulphide is sulphated and dissolved, moving the said other sulphide from the point in the sulphating material where the one sulphate was dissolved to parts of the material having greater and greater strength until a part is reached where the strength is sufficient to attack the said other sulphide, sulphating and dissolving the said other sulphide in that part of the material where it was thus attacked, whereby the two sulphates are separated in the sulphating material, withdrawing the two separated sulphates from their respective parts of the material, treating the separated sulphates for the recovery of their respective metal values with the consequent liberation of the acid-forming parts of the sulphates, and introducing said acid-forming parts into the sulphating mate-

rial wherever needed to maintain the acid strength thereof.

20. The herein described method which comprises maintaining a flowing stream of liquid sulphating material the acid strength of which increases in the direction of the source of the stream, introducing a mixture containing two sulphides in finely divided condition into said stream, sulphating that sulphide which is the more susceptible to the acid attack and dissolving its sulphate in the stream, moving the remaining and more resistant sulphide up the stream beyond the point where the said sulphate was dissolved until it reaches a point when the liquid is strong enough to attack it and then sulphating the latter sulphide and dissolving its sulphate in the stream, whereby the sulphates are separated in the stream and made available for separate treatment for the recovery of their respective metal values.

21. The herein described method which comprises maintaining a flowing stream of liquid sulphating material the acid strength of which increases in the direction of the source of the stream, introducing a mixture of two sulphides in finely divided condition into said stream, sulphating that sulphide which is the more susceptible to the acid attack and dissolving its sulphate in the stream, flowing said dissolved sulphate down the stream, moving the remaining and more resistant sulphide up the stream from the point of its introduction until it reaches a point when the liquid is strong enough to attack it and then sulphating the latter sulphide and dissolving its sulphate in the stream, whereby the sulphates are separated in the stream, treating the separated sulphates for the recovery of their respective metal values, and injecting the acid contents of the sulphates into the stream to move the more resistant sulphide therein and to maintain the sulphating strength of the liquid.

22. The herein described method which comprises maintaining a flowing stream of liquid sulphating material, introducing a mixture of copper sulphide and iron sulphide in the form of  $FeS_2$  into the stream, said sulphides being in a finely divided condition, moving the copper sulphide in the stream into a zone where the strength of the sulphating material is sufficient to convert it into the sulphate of copper, dissolving the sulphate of copper and removing it from the stream, removing the  $FeS_2$  from the stream and heating it to convert it into  $FeS$ , introducing the  $FeS$  into the copper sulphate to convert the latter into  $FeSO_4$  and  $CuS$ , removing the  $CuS$ , treating the  $FeSO_4$  to form  $Fe_2(SO_4)_3$  and introducing the latter into the stream.

23. The herein described method which comprises maintaining a body of acidulated sulphating material in liquid form the acid strength of which varies from point to point

in the body, introducing mixed sulphide ores in comminuted condition into said body at a point where the acid strength is relatively weak, moving said ores within the body until the various sulphides reach respective points when the acid is strong enough to attack and sulphate them, whereby the sulphates are separated in the body, dissolving the sulphates at the points where they were thus formed, withdrawing a sulphate from the body, treating the withdrawn sulphate to obtain sulphuric anhydride, and introducing into the body such part of the sulphuric anhydride as is required to maintain its acid strength.

24. The herein described method which comprises maintaining a flowing stream of liquid sulphating agent the acid strength of which increases in the up-stream direction, introducing a mixture of sulphide materials into said stream adjacent its lower end, said materials being in comminuted condition and containing copper sulphide and  $FeS_2$ , moving the various sulphides up-stream until they reach parts of the agent which are respectively strong enough to attack and sulphate certain of them except the  $FeS_2$ , withdrawing a sulphate from the stream and treating it to obtain  $SO_3$ , removing the  $FeS_2$  from the stream and heating it to form  $FeS$ , withdrawing the copper sulphate from the stream, introducing  $FeS$  into the copper sulphate to precipitate the copper content as  $CuS$ , introducing part of the  $SO_3$ , produced as above, and air into the  $CuS$  to change the latter to  $CuSO_4$ , and introducing the remaining part of the  $SO_3$  into the stream to strengthen the acid content thereof.

25. The herein described method which comprises maintaining a flowing stream of liquid sulphating agent the acid strength of which increases in the up-stream direction, introducing a mixture of sulphide materials into said stream adjacent its lower end, said materials being in comminuted condition and containing copper sulphide and  $FeS_2$ , moving the various sulphides up-stream until they reach parts of the agent which are respectively strong enough to attack and sulphate certain of them except the  $FeS_2$ , withdrawing a dissolved sulphate from the stream and treating it to obtain  $SO_3$ , removing the  $FeS_2$  from the stream and heating it to form  $FeS$ , withdrawing the dissolved  $CuSO_4$  from the stream, introducing  $FeS$  into the  $CuSO_4$  to form  $FeSO_4$  and precipitate the  $Cu$  as  $CuS$ , introducing part of the  $SO_3$ , produced as above, and air into the  $CuS$  to change the latter to  $CuSO_4$ , treating the  $FeSO_4$  to produce  $Fe_2(SO_4)_3$  and introducing the  $Fe_2(SO_4)_3$  and other parts of the  $SO_3$  into the stream to maintain the acid strength thereof.

GEORGE CAMPBELL CARSON.